

Patented Jan. 19, 1954

2,666,588

# UNITED STATES PATENT OFFICE

2,666,588

## FLOTATION PROCESS FOR SEPARATION OF SILICA AND RHODONITE

Carl H. Schack, Salt Lake City, Utah, and Karl C. Dean, Mexico City, Mexico, assignors to the United States of America as represented by the Solicitor of the Department of the Interior

No Drawing. Application December 15, 1952,  
Serial No. 326,172

6 Claims. (Cl. 241—20)

(Granted under Title 35, U. S. Code (1952),  
sec. 266)

1

The invention described herein may be manufactured and used by or for the Government of the United States for governmental purposes without the payment to us of any royalty thereon in accordance with the provisions of the act of April 30, 1928 (Ch. 460, 45 Stat. L. 467).

This invention relates to a process for the concentration of manganese ores, and, more particularly, to a froth flotation process for the separation of silica from rhodonite ores.

Manganese concentrates to be readily marketable should contain at least 33 per cent manganese. Rhodonite, a manganese silicate, in purest form contains a theoretical 42.4 per cent manganese, but, in the form in which it usually occurs in nature, contains a somewhat lower percentage. For example, the rhodonite content of a typical ore contained 38.1 per cent manganese. This ore also contained sulfides and silica minerals as well as the rhodonite and analyzed only about 20 per cent of manganese. This ore can be concentrated by sink and float procedure to 26.0 to 29.0 per cent manganese. Flotation of the contained sulfides from the manganese raises the concentration of the manganese to only about 30 per cent. Accordingly, separation of some of the contained silica is necessary to achieve a satisfactory grade of manganese concentrate. However, attempts to remove silica from this material by use of known flotation methods have not resulted in production of a satisfactory grade and satisfactory recovery of manganese values.

Accordingly, an object of this invention is to provide an improved flotation method for separation of silica and rhodonite.

Another object of this invention is to provide a combination of reagents that allows a satisfactory separation of silica and rhodonite.

A further object of this invention is to provide a flotation process for separation of silica from rhodonite whereby a rhodonite concentrate containing very little free silica and a silica concentrate containing very little manganese are obtained.

These and related objects and advantages of the invention hereinafter apparent as the ensuing description proceeds are accomplished by this invention which comprises adding to a pulp of rhodonite-silica containing material a suitable frothing agent, dextrine and tri-sodium phosphate, adjusting the pH to approximately 7.0, and floating off the silica from the rhodonite by staged additions of a suitable cationic reagent.

The use of tri-sodium phosphate in the combination of flotation reagents used for flotation of silica from rhodonite greatly enhances the selectivity of the silica flotation and at the same

time permits using a such smaller amount of expensive cationic-type collector and a shorter period of flotation. The theory of the reactions whereby the improvement in separation is obtained by the use of sodium phosphate is not definitely known. Flotation is a complex art in which little is known of the mechanisms whereby the flotation reagents, often in complex combinations and in minute quantities, accomplish the selective separations. In the present instance, the tri-sodium phosphate in combination with the other reagents either activates the silica minerals, quartz, etc., or it depresses the rhodonite. The action in either instance may be a chemical reaction, a physicochemical reaction, or a simple, or complex adsorption.

The rhodonite ore may be first ground to a suitable degree of fineness, although the invention is not dependent upon any particular limits in this respect. Ores ground to 48 mesh, minus 65 mesh, and minus 100 mesh have been satisfactorily employed.

If sulfides are present in the ground ore, they may first be floated by conventional methods. Most rhodonite ores contain a variety of sulfide minerals including galena, sphalerite, and pyrite and several siliceous minerals, chiefly rhodonite, quartz, chalcedony and opal. The separation of these sulfide minerals by flotation from the siliceous minerals is well known procedure. The resulting concentrate is then treated for silica removal by the process of this invention in its entirety or it may be screened into two or more fractions with flotation of silica from each of these fractions. The ore may also be deslimed and only the sand fraction floated.

Any standard frothing agent, such as the higher alcohols, pine oil, cresylic acid, B-23 frother, or others having no adverse effect on the selectivity of the collecting agents may be employed in the process. B-23 is a frothing agent composed of a mixture of high boiling point alcohols. Likewise, any of a number of known cationic collecting agents for silica flotation may be employed. Of these collecting agents lauryl amine hydrochloride, known commercially as E. P. 487 is preferred. Flotation from a substantially neutral pulp is preferred. The pH may be adjusted by the addition of sulfuric acid to the normally alkaline pulp. To illustrate the importance of pH adjustment, a test run utilizing a cationic collector known commercially as "Armac 12D" (the acetate salt of dodecyl amine) and an alkaline pH of 8.4, the natural pH of the ore ground in the water available, did not produce the favorable results of the invention.

The invention will be further illustrated but is not intended to be limited by the following examples of practice.

**3**  
**EXAMPLE I**

A lead-zinc-manganese ore containing the minerals galena, sphalerite, silica, and rhodonite primarily and assaying 26.5 per cent manganese was ground in an iron ball mill in five 4-minute stages through 100-mesh. The sulfides were

Essentially the same procedure was used in this second example as was used in Example I, with the exception that ore was ground to only minus 65-mesh and manganese content of the ore was higher.

*Table 2.—Reagent consumption in pound per ton of ore*

|                           | Time, minutes   | Z-6  | B-23  | K-101 | CuSO <sub>4</sub> | Na <sub>3</sub> PO <sub>4</sub> | Dextrene | H <sub>2</sub> SO <sub>4</sub> | E. P. 487 |
|---------------------------|-----------------|------|-------|-------|-------------------|---------------------------------|----------|--------------------------------|-----------|
| Bulk sulfides.....        | 5               | 0.15 | 0.056 | 0.50  | 0.15              |                                 |          |                                |           |
| +65+270 silica concs..... | 7 $\frac{1}{2}$ | .056 |       |       |                   | 0.90                            | 0.50     | 0.50                           | 0.22      |
| -270 silica concs.....    | 7 $\frac{1}{2}$ | .056 |       |       |                   | 1.00                            | .50      | .40                            | .10       |

floated by using normal sulfide reagents, namely: Z-6 xanthate (potassium pentasol amyl xanthate), K-101 (ammonium thiocyanate), B-23 frother, and CuSO<sub>4</sub>. The tails from this flotation were then removed from the cell and screened into a plus 270-mesh fraction and a minus 270-mesh fraction. These fractions were then floated separately in a mechanical flotation machine at approximately 30 per cent solids. B-23 was added to the pulp as a stabilizing frother in the amount of 0.056 pound per ton of ore, dextrene in the amount of 0.80 pound per ton and trisodium phosphate in the amount of 0.50 pound per ton were then mixed together in warm water and added to the cell, pH was then corrected downward from the pH of 8.4 used for sulfide flotation to a pH of 7.3. Small staged amounts of E. P. 487 cationic collector were then added to float the successive silica concentrates. With the exception of varying amounts of reagents, the flotation of both the plus 270- and the minus 270-mesh fractions was identical.

|                                  | Products | Weight, percent | Assay, percent Mn | Distribution, percent Mn |
|----------------------------------|----------|-----------------|-------------------|--------------------------|
| Bulk sulfides.....               |          | 6.7             | 9.5               | 2.2                      |
| +270 SiO <sub>2</sub> No. 1..... |          | 5.6             | 9.6               | 1.8                      |
| +270 SiO <sub>2</sub> No. 2..... |          | 4.3             | 12.1              | 1.8                      |
| +270 SiO <sub>2</sub> No. 3..... |          | 3.8             | 25.1              | 3.2                      |
| +270 Mn tail.....                |          | 43.3            | 35.8              | 52.4                     |
| -270 SiO <sub>2</sub> No. 1..... |          | 3.3             | 28.1              | 3.1                      |
| -270 SiO <sub>2</sub> No. 2..... |          | 9.8             | 26.1              | 8.7                      |
| -270 SiO <sub>2</sub> No. 3..... |          | 8.3             | 31.3              | 8.8                      |
| -270 Mn tail.....                |          | 14.9            | 35.7              | 18.0                     |
| Calculated head.....             |          | 100.0           | 29.56             | 100.0                    |

**EXAMPLE III**

This example is submitted solely to show the difference in results obtained from a test run previous to the time Na<sub>3</sub>PO<sub>4</sub> was used in testing and which duplicates the test shown in Example I, except for varying the reagents. Note should be taken of the reduced amount of E. P. 487 needed in the test where Na<sub>3</sub>PO<sub>4</sub> was used.

*Table 3.—Reagent consumption in pound per ton of ore*

|                                     | Time, minutes | Z-6  | B-23  | K-101 | CuSO <sub>4</sub> | H <sub>2</sub> SO <sub>4</sub> | E. P. 487 | Dextrene |
|-------------------------------------|---------------|------|-------|-------|-------------------|--------------------------------|-----------|----------|
| Bulk sulfides.....                  | 5             | 0.15 | 0.056 | 0.50  | 0.15              |                                |           |          |
| +100+270 SiO <sub>2</sub> conc..... | 10            | .056 | .056  |       |                   | .05                            | 0.40      | 0.60     |
| -270 SiO <sub>2</sub> conc.....     | 10            | .056 | .056  |       |                   | .40                            | .17       | 1.0      |

Reagent consumption and test results are shown in the following tables.

*Table 1.—Reagent consumption in pound per ton of ore*

|                            | Time, minutes   | Z-6  | B-23  | K-101 | CuSO <sub>4</sub> | Na <sub>3</sub> PO <sub>4</sub> | Dextrene | H <sub>2</sub> SO <sub>4</sub> | E. P. 487 |
|----------------------------|-----------------|------|-------|-------|-------------------|---------------------------------|----------|--------------------------------|-----------|
| Bulk sulfides.....         | 5               | 0.15 | 0.056 | 0.50  | 0.15              |                                 |          |                                |           |
| +270 silica flotation..... | 7 $\frac{1}{2}$ | .056 |       |       |                   | 0.50                            | 0.80     | 0.40                           | 0.15      |
| -270 silica flotation..... | 7 $\frac{1}{2}$ | .056 |       |       |                   | .50                             | 1.00     | .40                            | .15       |

*Table 1A*

| Products                         | Weight, percent | Assay, percent Mn | Distribution, percent Mn |
|----------------------------------|-----------------|-------------------|--------------------------|
| Bulk sulfide concentrate.....    | 7.6             | 9.5               | 2.7                      |
| +270 SiO <sub>2</sub> No. 1..... | 6.7             | 9.5               | 2.4                      |
| +270 SiO <sub>2</sub> No. 2..... | 4.7             | 11.3              | 2.0                      |
| +270 SiO <sub>2</sub> No. 3..... | 4.4             | 16.9              | 2.8                      |
| +270 Mn tail.....                | 31.3            | 35.3              | 41.4                     |
| -270 SiO <sub>2</sub> No. 1..... | 8.2             | 26.1              | 8.0                      |
| -270 SiO <sub>2</sub> No. 2..... | 9.5             | 24.3              | 8.6                      |
| -270 SiO <sub>2</sub> No. 3..... | 13.0            | 28.1              | 13.7                     |
| -270 Mn tail.....                | 14.6            | 33.6              | 18.4                     |
| Calculated head.....             | 100.0           | 26.69             | 100.0                    |

*Table 3A*

| Products                         | Weight, percent | Assay, percent Mn | Distribution, percent Mn |
|----------------------------------|-----------------|-------------------|--------------------------|
| Bulk sulfide conc.....           | 8.2             | 10.7              | 3.3                      |
| +270 SiO <sub>2</sub> No. 1..... | 10.2            | 16.4              | 6.3                      |
| +270 SiO <sub>2</sub> No. 2..... | 12.0            | 23.1              | 11.3                     |
| +270 Mn tail.....                | 21.7            | 34.1              | 28.0                     |
| -270 SiO <sub>2</sub> No. 1..... | 11.5            | 26.4              | 11.5                     |
| -270 SiO <sub>2</sub> No. 2..... | 6.0             | 24.7              | 5.6                      |
| -270 SiO <sub>2</sub> No. 3..... | 9.8             | 27.0              | 10.0                     |
| -270 Mn tail.....                | 19.7            | 32.3              | 24.0                     |
| Calculated head.....             | 100.0           | 26.46             | 100.0                    |

75 A comparison of the foregoing examples clearly

illustrates the advantages to be gained by the use of tri-sodium phosphate in combination with the other reagents utilized for separation of silica. Thus, in the test of Example III, ten minutes were required to float the silica minerals from each of the two sized fractions and a total of 0.77 pound of collector (E. P. 487) was used per ton of ore treated. The combined manganese products, plus the minus 270-mesh Mn tail, represented a recovery of 52 per cent of the manganese and assayed 33.3 per cent manganese. Example I is an exact duplicate test of Example III, except that tri-sodium phosphate was used. In this test only 7½ minutes were required to float each of the two sized fractions and a total of only 0.30 pound of collector (E. P. 487) was used per ton of ore treated. At the same time a recovery of 59.8 per cent of the manganese was made in a product assaying 34.0 per cent manganese. Comparison of the data from the two examples show that the use of tri-sodium phosphate decreases the time needed to float the silica minerals, reduces the amount of collector needed to less than half, and at the same time, improves both the grade of the final product and the overall recovery of the manganese.

It will be appreciated from a reading of the foregoing specification that the invention herein described is susceptible of various changes and modifications without departing from the spirit and scope thereof.

What is claimed is:

1. A process for the froth flotation of silica from rhodonite comprising adding to a pulp of rhodonite-silica containing material a frothing agent, dextrine, and tri-sodium phosphate, adjusting the pH of the pulp to about 7, and floating the silica from the rhodonite by addition of a cationic collecting agent.

2. A process for the concentration of rhodonite ores comprising grinding the ore, separating the sulfides from the siliceous minerals, adding to a pulp of the resulting siliceous mineral concentrate a frothing agent, dextrine, and trisodium phosphate, adjusting the pH of the pulp to about 7, and floating the silica from the rhodonite by addition of a cationic collecting agent.

3. A process for the concentration of rhodonite ores comprising grinding the ore, separating the sulfides from the ground ore by froth flotation, adding to a pulp of the resulting siliceous mineral concentrate a frothing agent, dextrine, and tri-sodium phosphate, adding sulfuric acid to neutralize the pulp, adding a cationic collecting agent to the pulp, and floating the silica from the rhodonite.

4. A process for the concentration of rhodonite ores comprising grinding the ore to at least past 48 mesh, separating the sulfides from the ground ore by froth flotation, separating the resulting siliceous mineral concentrate into at least two size fractions, adding to a pulp of each fraction a frothing agent, dextrine and trisodium phosphate, neutralizing the pulp with sulfuric acid, adding a cationic collecting agent to the neutralized pulp, and floating the silica from the rhodonite.

5. A process for the froth flotation of silica from rhodonite comprising adding to a pulp of rhodonite-silica containing material a frothing agent, dextrine and a small amount of trisodium phosphate, neutralizing the pulp with sulfuric acid, and floating the silica from the rhodonite by staged additions of lauryl amine hydrochloride.

6. A process for producing a manganese concentrate from a lead-zinc-manganese ore containing the minerals galena, sphalerite, silica, and rhodonite comprising grinding the ore, separating the sulfide minerals from the ground ore by froth flotation, preparing a pulp of the siliceous minerals, adding to the pulp a stabilizing frothing agent, dextrine, and a small amount of trisodium phosphate, adjusting the pH of the pulp to approximately 7 by addition of sulfuric acid, and floating the silica from the rhodonite by additions of lauryl amine hydrochloride between flotation stages.

CARL H. SCHACK.  
KARL C. DEAN.

References Cited in the file of this patent

U. S. Bureau of Mines Report of Investigations, RI 3842, February 1946, and RI 445, April 1949. (Copies available in Scientific Library.)